

Sept. 11, 1934.

E. J. JOHNSON

1,972,996

SHOT SHELL AND PROCESS OF MAKING SAME

Filed July 18, 1931

3 Sheets-Sheet 1



INVENTOR  
*Edwin J. Johnson,*  
BY

*J. O'Connell*  
ATTORNEY

Sept. 11, 1934.

E. J. JOHNSON

1,972,996

SHOT SHELL AND PROCESS OF MAKING SAME

Filed July 18, 1931

3 Sheets-Sheet 2



FIG. 2

INVENTOR  
*Edwin J. Johnson*  
BY  
*J. D. O'Connell*  
ATTORNEY.

Sept. 11, 1934.

E. J. JOHNSON

1,972,996

SHOT SHELL AND PROCESS OF MAKING SAME

Filed July 18, 1931 3 Sheets-Sheet 3

Fig. 6.



Fig. 7.



Fig. 8.

Fig. 9.

Inventor

Inventor



३४

J. O'Connell Attorney

## UNITED STATES PATENT OFFICE

1,972,996

SHOT SHELL AND PROCESS OF MAKING  
SAMEEdwin J. Johnson, Montreal, Quebec, Canada,  
assignor to Canadian Industries Limited,  
Montreal, Quebec, Canada, a corporation of  
Canada

Application July 18, 1931, Serial No. 551,779

27 Claims. (Cl. 102—16)

This invention relates to shot shells and processes of making same, and it comprises a waterproofed shot-shell, having a paper tube body impregnated to the outer surface with a waxy material, such as paraffin, ceresin, ozokerite and the like, the surface of said paper body being uniformly and substantially free from a film of unabsorbed wax and provided with a hard, dry, cohesive sheath produced from an applied pyroxylin composition; and it further comprises a process of producing such a waterproofed paper shot shell by impregnating said paper tube with wax, removing superficial wax by mechanical action to produce a uniform surface free from a film of unabsorbed wax and applying to said film-free surface a pyroxylin composition and allowing the same to dry and harden; all as more fully hereinafter set forth and as claimed.

This application contains subject matter common to applicant's prior co-pending applications Serial Nos. 92,594 and 264,967 of which applications the present case is a continuation in part.

The main object achieved in the present invention is the manufacture of shot shells which are thoroughly moisture proof and are unaffected by atmospheric conditions, which can be fired in rapid succession from a gun without tending to stick in the hot barrel, which do not tend to stick in the breech, which are strong, durable and sufficiently rigid to withstand the rough usage to which shot shells are usually subjected in and out of the gun, and which are at the same time sufficiently elastic to allow for the necessary degree of expansion upon firing without liability to rupture.

Shot shell tubes are usually made of cardboard or heavy paper; often without any particular treatment. It is recognized that absorption of moisture by these tubes creates difficulties of various kinds; and particularly swelling. With the accurate mechanism of a good gun the permissible variation in size is very little. Any substantial absorption of moisture and swelling may render it difficult or impossible to handle a shell by the gun mechanism. Various ways of waterproofing shells and protecting them against rain, snow and atmospheric conditions have been proposed, but not found satisfactory in practice; largely because of other difficulties arising. A shot shell tube must be quite rigid and yet have a certain degree of elasticity to fulfill the requirements of firing in magazine guns. It is not permissible to use any waterproofing composition materially affecting these properties.

In brief, my process of waterproofing shot shells comprises impregnating a paper shot shell tube

with wax, removing the film of superficial wax at elevated temperatures by mechanical action, (including within this term removal by chemical action and by rubbing, brushing, wiping, dissolving, tumbling and absorbing operations) and finally applying to the film-free surface so produced a pyroxylin lacquer of special composition. In order to exemplify my process, a specific example of its application will be described.

In the production of waterproofed shot-shells several pieces of mechanical equipment are useful. These will be briefly described in connection with the accompanying drawings. In this showing:

Fig. 1 is a front elevation of a rotary drier or wax removing device with rotating shaft and heating coils shown in dotted lines.

Fig. 2 is a longitudinal section through the wax removing device along the line 2—2 of Fig. 3, parts being shown in elevation.

Fig. 3 is a plan view, a section being taken along the line 3—3 of Fig. 2 to show the construction of the rotary shaft.

Fig. 4 is an end view of a sawdust rumbler, shown in elevation.

Fig. 5 is a front elevation of the rumbler.

Fig. 6 is a side elevation of a dipping or coating machine.

Fig. 7 is a plan view of the coating machine, while

Figs. 8 and 9 show details of a shot-shell rack for holding shells in the coating machine during operation.

In the figures like numerals refer to like structures. Figs. 1, 2 and 3 show details of a structure suitable for removing superficial wax from paraffin impregnated shot-shell paper tubes. The structure of this wax removing device is essentially that of a rotary drier. A hopper 1 is employed for introducing the paper tubes, usually cut to shot-shell length, into the rotating shaft 2, of the device. This shaft 2 runs through two chambers, 11 and 17. The first chamber 11 is a heating section, heat being supplied by the coils of pipe 12 and 13 which surround the rotating shaft on all sides. The rotary shaft of the drier is perforated in four series of holes, 3, 4, 5 and 6 which allow any melted wax to drip into the receiving pans 14. Access to these pans is provided by the hinged doors 15 shown in Fig. 1.

In chamber 17 of the wax removing device the paper shot-shell tubes are subjected to treatment with air which blows against them at a high velocity. Air is blown into the lower end of the rotary shaft 2 by means of the fan 19. This fan 19 may be driven by a belt (not shown) operat-

ing on the pulley 25 which is mounted on a base 22. The pressure side, 21 of the fan enters the lower end of the shaft 2. The air blown in passes out of the shaft 2 through the perforations 7 and 5 into the chamber 17. It then passes over the heating coils 18 and enters the suction side of the fan 20. The heated air is thus recirculated and serves to blow off any wax which may be left adhering to the paper tubes.

- 10 After passing through the rotary shaft 2 the paper shot shell tubes are discharged from a trap door, not shown, at the lower end of the shaft and into the discharge spout 32. The trap door is opened once during every revolution of the shaft 15 2, being closed thereafter to prevent the escape of the heated air inside the shaft. The paper tubes are caught in a barrel which is placed beneath the spout 32.

The rotating shaft 2 of the wax removing device is provided with a spiral baffle or a worm 16, the structure of which is shown best in Fig. 3. This worm serves to propel the paper tubes through the rotary shaft.

After the removal of the superficial wax in the 25 wax removing device, the paper tubes are introduced into a rumbler shown in Figs. 4 and 5. This rumbler may consist of an octagonal shaped drum 26 mounted on a shaft 8 and driven by a belt 34. A hand-wheel 31 is provided at the other end of 30 shaft 8. Sawdust and paper tubes are introduced into the drum 26 through a trap door, not shown. After rumbling is completed the trap door is opened and the mixture of sawdust and tubes is 35 discharged into the lower part of the device. The baffles 9 serve to direct the mixture into a screened tray 29. The perforations in the bottom of the screened tray 29 serve to discharge the sawdust but retain the paper tubes, the sawdust falling into the receiver 30.

10 Lacquering is accomplished by means of the coating machine shown in Figs. 6 and 7. The working parts of this machine consist essentially of two endless, motor driven sprocket chains 35-35. These chains follow a circuitous path 15 around the sprockets 44, 40, 45, 46 and 47. A dipping well 39 is provided below the sprocket 40. This well is filled with a suitable lacquer composition which is kept at a constant level by means of the overflow 48. Fresh lacquer is continually 20 pumped from the reservoir 49 and through the pump 50 into the well 39. Upon overflowing, it returns to the reservoir 49. A float 51 is provided in the reservoir to serve as a warning when the supply of lacquer becomes depleted. The sprocket 25 chains 35-35 are driven by means of the motor 36, the reduction gearing 37 and the chain 38, while the pump is driven by the chain 53.

In order to point out more specifically the details of my process I will now describe the manufacture of waterproof shot-shells in more detail, 30 the description including the operation of the various devices described above.

The first step in the process of making the paper tubes for shot-shells comprises rolling the paper into the form of tubes on a mandrel. The paper is coated on both sides with a paste as it passes through a pasting machine prior to rolling. In this process the composition of the paste is important. Not more than one part of wax to 35 128 parts of starch should be employed. A simple composition for this paste is as follows:

|                |           |
|----------------|-----------|
| Starch-----    | 2 pounds  |
| Japan wax----- | 1/4 ounce |
| 75 Water ----- | 10 quarts |

Upon boiling, the above composition forms a thick paste which coats the paper with a gelatinous layer. This dries to a strong, hard flexible coat that is difficult to remove and which passes 80 the sizing operation without rupture. After pasting and rolling, the tubes are dried and seasoned in a damp atmosphere before sizing. The sizing operation is carried out in a machine which automatically puts the tubes on a mandrel and pushes both tubes and mandrel through the die so that the resulting tubes have a definite diameter falling between certain prescribed limits. This diameter amounts to 0.787 inch for 12 gauge tubes, for example.

The wax employed in the paste is required as a lubricant during the sizing operation. If a small proportion is not used the paper tubes usually 90 crumple up on the mandrel and are rendered useless. The size of the die through which the paper tubes are pressed determines whether the sizing is "hard" or "soft". Hard sized tubes have a high gloss on their surface, while soft sized tubes have a dull surface appearance. The "hardness" of the sizing determines to a large extent the rapidity of wax absorption during a 100 later step of the process.

After sizing, the tubes are cut in an automatic machine into short cylinders of a length suitable for assembly into the shot-shell. A 12 gauge shell, for example, requires a paper tube with a length, 105 when cut, of 2 1/4 inches. After cutting approximately to length the paper tubes are ready for impregnation with wax.

Various kinds of wax may be employed, such as ceresin and ozokerite, but I have found that 110 a high grade paraffin wax having a melting point lying between 123° to 126° F. and having a low oil content is advantageous. The wax is placed in a tank, melted and raised to a temperature of 180° to 190° F. before the paper tubes are 115 dipped. The paper tubes are placed in a wire basket and immersed for from one to two hours in the bath of molten wax, depending on the rate of wax absorption. The bath of wax may be thermostated in order to maintain a constant temperature and a uniform product.

It has been found that the paper tubes prepared as described tend to absorb wax longitudinally from the ends rather than laterally from the surfaces. The progress of the films of wax, 125 entering from the ends, may be readily observed by splitting open the tubes and separating into layers. The parts which contain wax appear much darker than those parts which the wax has not yet reached.

Prior to the development of my process it was the practice to allow the paper tubes to remain in a bath of wax for a short time after they had become completely saturated. In this case, even after subsequent heating and draining treatments 135 to remove wax, the wax content was still from 20 to 25 per cent of the total weight of the waxed tube. In my present process, however, the paper tubes are advantageously withdrawn from the bath sometime before the wax films which approach each other from opposite ends of the paper tubes have met. If the paper tubes are withdrawn when there is a space amounting to 1/4 to 1/2 inch still remaining between these wax films, best results are obtained. Such tubes, after subsequent treatment to remove the film of superficial wax, have a wax content approximating 16 to 18 per cent by weight, the wax content having been thoroughly homogenized during the wax removal and rumbling operations.

80

85

90

95

100

105

110

115

120

125

130

135

140

145

150

- In the wax impregnation process the temperature of the bath is important. If the temperature falls much below 180° F. the rate of absorption is low and a larger proportion of wax is obtained in the finished tubes, while, if the bath rises much above 190° F., there may ensue an objectionable cooking or baking of the paste which is present between the layers of paper. The paste tends to lose its adhesiveness. It is obvious, of course, that the temperature of the bath must be kept well below the point at which the paper tends to char. The tubes impregnated at a low temperature tend to exude wax even after the final treatment for wax removal.
- It is important to maintain the paper tubes somewhat under-saturated for best results. It is also advantageous to cut the tubes to cartridge length before the wax impregnation. As mentioned previously the wax is mostly absorbed longitudinally from the ends of the tubes. If the tubes are long they tend to become under-saturated at the center and super-saturated at the ends. Uniformity of impregnation is thus difficult. A considerable saving of time also results from the cutting of the tubes. This cutting to length prior to impregnation with wax constitutes an important step in my new process.
- Of course the cutting of the paper tubes to shot-shell length prior to impregnation with wax and the withdrawal of the tubes from the impregnating bath prior to complete saturation are manufacturing refinements which are not essential to the production of satisfactory shot-shells. As described in my copending application, Serial No. 264,967, filed March 26, 1928, impregnation with paraffin may be by dipping, coating, spraying and the like. But it is preferable to use only about 18 per cent by weight of the paraffin in the paper containers.
- After the tubes are impregnated with wax, they are dumped into the hopper of the wax removing device shown in Figs. 1, 2 and 3, described previously. The rotation of the shaft 2 of this device is controlled to 3 to 4 revolutions per minute. The shaft of the device is tilted at an angle of 2 or 3 degrees to the horizontal to facilitate the passage of the tubes through the chambers 11 and 17. The length of the shaft is about 15 feet and the paper tubes are conveyed through it and ejected in about 12 minutes. The temperature of the heating section 11 is maintained at about 220° to 240° F. while the air blowing through chamber 17 is maintained at about the same temperature. This air is circulated over the paper tubes in the latter chamber at the rate of about 250 cubic feet a minute. It may be said that this air exerts a "wiping" action on the tubes.
- When discharged from the wax removing device, the paper tubes have the appearance of being free from superficial wax. However, they sometimes still possess a film of wax over the surface, the surface layers showing a higher wax content than the inner layers. It is necessary to remove this wax film in order to successfully lacquer the paper tubes. This film of wax may be sufficiently removed by rumbling in sawdust, for example.
- The rumbling operation is conducted in the device shown in Figs. 4 and 5, described previously. The rumbler is rotated at approximately 24 revolutions per minute and from 15 to 20 minutes. The sawdust used in this rumbling operation is heated to a temperature of from 180° to 190° F. by means of an auxiliary oven, not shown, prior to introduction into the rumbler. About  $\frac{1}{4}$  barrel of this hot sawdust is introduced to 1 barrel of paper tubes. Soft wood sawdust is employed, which may be screened to remove coarse chips as well as fine dust. When fresh, the sawdust must be dried to reduce its moisture content to from 4 to 8 per cent. The sawdust can be re-used several times in the rumbling operation, being reheated between each operation. When the wax content of the sawdust reaches a maximum of about 8 per cent of wax it should be discarded. The actual amount of wax removed in the rumbling operation is small, amounting to only about 0.03 per cent of the weight of the tubes treated.
- The rumbling operation consists essentially in a mechanical removal of the surface film of wax. The hot sawdust directly absorbs or "blots" the wax from the surface upon contact with the tubes. It also mechanically rubs and scours wax from the surface. Various other mechanical methods for removing the surface film of wax are possible provided rubbing, scouring or blotting operations are included. It is also true that various other absorbent materials can be employed in place of sawdust in this operation, such as bran, paper scraps and the like. The film of wax may also be sufficiently removed by dissolving the same in a solvent such as gasoline. Such processes are included in the term "mechanically removing".
- Treatment of the wax impregnated paper tubes in the wax removing device of Figs. 1, 2 and 3, followed by rumbling in sawdust or the like, constitutes another refinement which may be regarded as my preferred method of preparing the tubes for the application of the pyroxylin coating composition. As described in my acknowledged copending application, Serial No. 264,967, removal of the superficial film of unabsorbed wax from the surface of the waxed tubes may be accomplished by heating the tubes to around 250° to 260° F. for a period of about nine minutes and agitating or spinning the shells in a centrifugal or other rotary device. Rinsing the shells with gasoline or the like to remove paraffin from surface fibers is likewise applicable. These mechanical methods of removing the superficial film of unabsorbed wax give satisfactory results.
- After the above described rumbling operation in what I consider the best embodiment of my invention, the paper shot shell tubes are assembled, the caps applied and they are loaded to produce an otherwise finished shell, by operations standard to shot-shell loading. The shells are now ready for application of the lacquer composition which is applied by dipping, the operation being conducted by means of the coating machine shown in Figs. 6 and 7. The shells are first mounted in detachable racks which may be similar to the rack shown in Fig. 8. A detail of a suitable end bracket for such racks is shown in Fig. 9. The shells are slipped through the holes 33 in the rack, being held in position by the rim of the cartridge base. The filled racks are inserted in the dipping machine and may be held in place by suitable slots 10, provided in the end brackets, as shown in Fig. 9. These slots in the end brackets are designed to cooperate with studs, not shown, which are mounted on the edges of the two endless sprocket chains 35—35 of the coating machine. The racks are thus held in position between the two sprocket chains. A filled rack is shown in position in Figs. 6 and 7 at 52. The motion of the sprocket chain serves to dip the paper tubes of the car-

tridges into the well containing coating composition at 39. After dipping, the cartridges are pulled upward along the drip pan 41 and finally travel horizontally towards the sprocket 46. The 5 racks of coated cartridges are removed from the coating machine at 43.

Altogether about 20 minutes is allowed for 10 draining and drying of the dipped shells before they are removed from the coating machine. The coating has, by that time, dried sufficiently to allow the shells to be dumped into boxes. During the latter part of their travel toward 15 43 the shells are maintained at a temperature of about 95° to 100° F. and the coating is fully dry and hard when they reach this point.

The shot-shells produced by the method described above are considerably more waterproof than any shells produced previous to the introduction of my process. For example, they are 20 30 to 40 times as waterproof as shells whose paper tubes have been merely impregnated with paraffin alone. While some shells coated with lacquer alone are fairly waterproof they are not uniformly so. Any rupture of the coating causes 25 a large decrease in their waterproofness. The average waterproofness is not high. Such lacquer coated shells are also commonly too brittle and are inclined to split during firing. Shells produced by my process are not only considerably 30 more waterproof but are also not brittle.

The combination of the wax impregnation on the inner layers of the paper shells with the lacquered coating on the outside appears to give the shot-shells certain highly desirable characteristics. The paraffin preserves or increases the natural elasticity of the paper tubes. There appears to be a true combination between the wax inner coating and the lacquer outer coating. The paraffin acts as a plasticizer, impregnating and softening the interior of the paper tube, while the lacquer acts as a strengthening agent on the outside, imparting stiffness and rigidity. There is thus a coaction between the two coatings which cooperate to produce the desired result. The 40 combination of the coatings is thus obviously not the mere sum or aggregation of the two coatings. The total weight of the coatings amounts to nearly  $\frac{1}{4}$  the weight of the paper tubes. The coatings thus form an important part of the shell 45 structure itself and are essential for the production of satisfactory shot-shells.

The fact that a pyroxylin lacquer can be made to adhere in cohesive engagement with a paper tube containing wax is indeed surprising. The 50 lack of adherence between a lacquer coating and a greasy or waxy surface has been so generally recognized that manufacturers of lacquer commonly place directions on containers to the effect that all traces of wax or grease must be removed prior to application of the lacquer. While there 55 has been at least one suggestion in the literature of coating a wax impregnated shot-shell with "celluloid varnish", all attempts to produce satisfactory shells in the manner there described have 60 proved to be futile. These prior coatings were 65 non-adherent. In fact, it is only by the use of my mechanical methods for removing the continuous superficial film of unabsorbed wax from the surface, combined with the pyroxylin compositions 70 which I employ, that success has finally been obtained.

The majority of lacquer compositions now on the market have at least a small content of hydrocarbon solvents, such as toluol. Such lacquer 75 compositions are not generally satisfactory in my

process unless they are modified by the inclusion of a drying oil, such as China wood oil. The hydrocarbon content apparently dissolves some paraffin from the paper shot-shells, producing a film of wax upon the surface of the lacquer. This film 80 prevents evaporation of the lacquer solvent, the lacquer frequently requiring several days to dry completely. When finally dried the surface is mottled in appearance and will craze and chip off easily. The inclusion of a drying oil, such as 85 China-wood oil, prevents these difficulties, provided the hydrocarbon content is not too great. It is advantageous, however, to employ a lacquer free from hydrocarbons in my process.

In the absence of hydrocarbon solvents in a 90 given lacquer composition, the addition of drying oils such as linseed, hemp and poppy oil will produce satisfactory results in my process, but China-wood oil appears to produce the best results. In any case, before applying the final 95 coat of lacquer, with or without a drying oil, it is necessary to remove the continuous surface film of unabsorbed wax from the wax impregnated paper tubes by the rubbing, wiping, blotting and other mechanical methods outlined previously. 100

As stated in my acknowledged copending application lacquers in general are satisfactory which are of pyroxylin composition, which are of resinous-pyroxylin composition, which contain a drying oil, which are free of hydrocarbon solvents, which contain a resin and a drying oil such as China-wood oil, and which contain a resin and a drying oil and are free from hydrocarbon solvents. 105

I have found that natural resins, such as copal, 110 dammar, etc., or ester guns are advantageous ingredients of lacquer compositions suitable for my process. I also advantageously add a drying oil to these compositions. Two specific examples of lacquer compositions suitable for my process 115 are as follows:

|                | Per cent |
|----------------|----------|
| Pyroxylin      | 11.2     |
| China-wood oil | 10.0     |
| Dammar         | 10.0     |
| Ethyl alcohol  | 120      |
| Ethyl acetate  | 16.2     |
| Butyl acetate  | 23.4     |
| Butyl alcohol  | 23.2     |
|                | 6.0      |
|                | 125      |
|                | 100.0    |

|                   | Per cent |
|-------------------|----------|
| Pyroxylin         | 11.2     |
| Diethyl phthalate | 3.7      |
| Blown linseed oil | 10.0     |
| Dammar            | 130      |
| Ethyl alcohol     | 6.3      |
| Ethyl acetate     | 15.0     |
| Butyl acetate     | 25.8     |
| Butyl alcohol     | 22.0     |
|                   | 6.0      |
|                   | 135      |
|                   | 100.0    |

Either of the above compositions applied to a wax impregnated paper tube, suitably treated by 140 my process, will dry in 15 to 30 minutes. Application of the lacquer may be by dipping or spraying. Pyroxylin compositions of the nature noted are stable and do not stick in a shotgun and, as a matter of fact, vanish under the extreme conditions of heat and pressure caused by rapid firing. 145

While I have specifically described my process as applied to the production of waterproof shot-shells, it is obvious that it is applicable to other 150

- technical uses. Paper tubes of various sorts and sizes can be so treated. The waterproofed tubes can be employed as containers for chemicals, foodstuffs and the like as well as for other purposes. In all cases it is desirable to cut the tubes to length in order that the wax may be able to penetrate more rapidly from the ends. It is only necessary to impregnate the tubes with wax at a temperature considerably above melting point 5 of the said wax, to remove the surface film of unabsorbed wax by rubbing, dissolving, wiping, blotting and other mechanical operations and to then apply the lacquer coat. It is advantageous to carry out the mechanical removal of the surface film of wax while heating the paper tubes. It is also desirable to somewhat under-saturate the tubes with wax during the impregnating operation, the wax becoming homogenized throughout the body of the paper tubes during subsequent 10 operations.
- This application is in part a continuation of my prior applications, Serial Nos. 92,594, filed March 5, 1926 and 264,967, filed March 26, 1928.
- What I claim is:
- 25 1. A process of treating shot shells which consists in impregnating paper shot shell tubes with paraffin subjecting the impregnated tubes to a temperature of approximately 250° to 260° F. for about nine minutes, and then applying to the 30 tubes a coating of pyroxylin composition.
2. An improved shot gun shell comprising a tubular, fibrous wax impregnated container, the waxed surface thereof being uniformly and substantially free of a film of unabsorbed wax, and 35 having a dry, hard, cohesive waterproof sheath produced from an applied pyroxylin composition containing a resin.
3. An improved shot gun shell comprising a tubular, fibrous wax impregnated container, the 40 waxed surface thereof being uniformly and substantially free of a film of unabsorbed wax, and having a dry, hard, cohesive waterproof sheath produced from an applied pyroxylin composition containing a resin and a drying oil such as China- 45 wood oil.
4. An improved shot gun shell comprising a tubular, fibrous wax impregnated container, the waxed surface thereof being uniformly and substantially free of a film of unabsorbed wax, and 50 having a dry, hard, cohesive waterproof sheath produced from an applied pyroxylin composition containing a resin and being free from hydrocarbon solvents.
5. An improved shot gun shell comprising a tubular fibrous wax impregnated container, the waxed surface thereof being uniformly and substantially free of a film of unabsorbed wax, and 55 having a dry, hard, cohesive waterproof sheath produced from an applied pyroxylin composition containing a resin and a drying oil and being free from hydrocarbon solvents.
6. In a shot shell, a uniformly wax-impregnated paper container having a fibrous mat surface and an outer sheath of resinous pyroxylin composition in locking engagement with said 60 surface.
7. An improved method of coating shot gun shells which comprises impregnating a paper container with wax, heating such wax impregnated 65 container to a temperature substantially above the melting point of the wax and under agitating conditions to produce a uniform waxed surface free of a film of unabsorbed wax and applying to said film-free surface a pyroxylin lacquer sub- 70 stantially free from hydrocarbon solvents, and allowing said lacquer to dry and harden.
8. An improved method of coating shot gun shells which comprises impregnating a paper container with wax, heating such wax impregnated 75 container to a temperature substantially above the melting point of the wax and under agitating conditions to produce a uniform waxed surface free of a film of unabsorbed wax and applying to said film-free surface a pyroxylin composition containing a resin and allowing the same to dry and harden. 80
9. An improved method of coating shot gun shells which comprises impregnating a paper container with wax, heating such wax impregnated 85 container to a temperature substantially above the melting point of the wax and under agitating conditions to produce a uniform waxed surface free of a film of unabsorbed wax and applying to said film-free surface a pyroxylin composition containing a resin and a drying oil and allowing the same to dry and harden. 90
10. An improved method of coating shot gun shells which comprises impregnating a paper container with wax, heating such wax impregnated 95 container to a temperature substantially above the melting point of the wax and under agitating conditions to produce a uniform waxed surface free of a film of unabsorbed wax and applying to said film-free surface a pyroxylin composition containing a resin and China-wood oil and allowing the same to dry and harden. 100
11. An improved method of coating shot gun shells which comprises impregnating a paper container with over 18 per cent by weight of wax, 110 heating such wax impregnated container at a temperature substantially above the melting point of such wax to reduce the paraffin content to about 18 per cent and under agitating conditions to produce a uniform waxed surface free 115 of a film of unabsorbed wax and applying to said film-free surface a coating of pyroxylin lacquer and allowing the same to dry and harden.
12. An improved method of coating shot gun shells which comprises making a wax-impregnated paper shell, superficially removing the wax by heating to a temperature above its melting point while agitating to produce a fibrous mat surface of uniform wax content and applying a 120 sheath of pyroxylin-resin composition in locking 125 engagement to said mat surface.
13. In the manufacture of shot shells, the steps which comprise impregnating paper shot shell tubes with wax and then mechanically removing any film of unabsorbed wax from the outer surface of the tubes to prepare said surface for the 130 application of a lacquer.
14. The process of claim 13 wherein the film of unabsorbed wax is mechanically removed by contacting said paper shot shell tubes with a 135 wax-absorbent material.
15. In the manufacture of shot shells the steps which comprise impregnating paper shot shell tubes with wax, heating such wax impregnated tubes to a temperature substantially above the 140 melting point of the wax and under agitating conditions to produce a uniform surface free from a film of unabsorbed wax and capable of firmly retaining an applied lacquer coating.
16. The process of claim 15 wherein the paper shot shell tubes are cut to length prior to impregnation with wax. 145
17. In the manufacture of shot shells, the steps which comprise impregnating paper shot shell tubes with wax, heating said tubes to a tempera- 150

ture substantially above the melting point of wax and mechanically removing any excess of unab-  
sorbed wax by a rumbling operation with a wax-  
absorbent material.

18. The process of claim 17 wherein the wax-  
absorbent material comprises sawdust.

19. In the manufacture of shot shells, the steps  
which comprise impregnating said tubes with  
molten wax, rendering uniform the wax content  
10 while heating under agitating conditions and me-  
chanically removing the superficial film of unab-  
sorbed wax, thereafter coating said paper tubes  
with a pyroxylin lacquer.

20. In the manufacture of shot shells, the  
15 process which comprises impregnating paper shot  
shell tubes with wax, mechanically removing any  
film of unabsorbed wax from the outer surface  
of the tubes and applying to said surface a lac-  
quer of pyroxylin composition.

21. The process in accordance with claim 20  
in which the lacquer contains a drying oil.

22. The process in accordance with claim 20  
in which the lacquer is substantially free from  
solvents for wax.

23. In the manufacture of shot shells, the  
process which comprises impregnating paper shot  
shell tubes with wax, removing the film of unab-  
sorbed wax from the outer surface of the tubes  
and coating said film-free surface with a pyroxy-  
lin composition containing a drying oil.

24. An improved method of coating shot gun  
shells which comprises impregnating a paper

shot shell tube with wax under conditions leav-  
ing a film of unabsorbed wax on the surface of  
the tube, treating the waxed surface of the tube  
with a solvent for the wax to remove from the  
surface the film of unabsorbed wax, and applying  
to the film-free surface a pyroxylin composition.

25. A shot shell comprising a paper tube uni-  
formly impregnated with wax to the outer sur-  
face, said surface being mechanically freed from  
a film of unabsorbed wax and provided with a  
hard, dry, cohesive sheath produced from an ap-  
plied pyroxylin composition.

26. A shot shell comprising a paper tube uni-  
formly impregnated with wax to the outer surface,  
said surface being uniformly and substantially  
free from a film of unabsorbed wax and pro-  
vided with a hard, dry, cohesive sheath produced  
from an applied pyroxylin composition; said sur-  
face having been mechanically freed from unab-  
sorbed wax by heating substantially above the  
melting point of the wax while under agitating  
conditions prior to application of said pyroxylin  
composition.

27. A shot shell comprising a paper tube uni-  
formly impregnated to its outer surface with about  
18 per cent of wax, said surface being uniformly  
and substantially free from a film of unabsorbed  
wax and provided with a hard dry cohesive sheath  
produced from an applied pyroxylin composition  
containing a resin and a drying oil.

EDWIN J. JOHNSON.